

# United States Patent [19]

Wu et al.

[11] 4,276,348

[45] Jun. 30, 1981

[54] HIGH TENACITY POLYETHYLENE FIBERS  
AND PROCESS FOR PRODUCING SAME

[75] Inventors: Wen-li Wu; William B. Black, both of  
Pensacola, Fla.

[73] Assignee: Monsanto Company, St. Louis, Mo.

[21] Appl. No.: 109,954

[22] Filed: Jan. 7, 1980

## Related U.S. Application Data

[62] Division of Ser. No. 848,168, Nov. 3, 1977, Pat. No.  
4,228,118.

[51] Int. Cl.<sup>3</sup> ..... D02G 3/00

[52] U.S. Cl. ..... 428/373; 57/243;

428/364

[58] Field of Search ..... 428/364, 359, 373;  
260/DIG. 23; 57/243

## [56] References Cited

### U.S. PATENT DOCUMENTS

2,210,774 8/1940 Perrin et al. ..... 526/352.2  
3,396,073 8/1968 Touey et al. ..... 428/369

## FOREIGN PATENT DOCUMENTS

215865 5/1957 Australia ..... 260/DIG. 23

## OTHER PUBLICATIONS

Porter et al., "Polymer Engineering and Science," Mar. 1976, vol. 16, No. 3 (pp. 200-203).

Porter et al., "Journal of Polymer Science," Polymer Physics Ed., vol. 16 (pp. 1729-1737), 1978.

Porter et al., J.P.S. vol. 13, 1177-1886.

Baranov et al., "Leningrad," vol. 17 (5), 1550-1552 (1973).

Primary Examiner—Lorraine T. Kendall

Attorney, Agent, or Firm—John W. Whisler

[57]

## ABSTRACT

Polyethylene yarns having tenacities of at least 12 grams per denier are produced at commercially feasible spinning speeds by a process in which a high density polyethylene having a  $M_n$  of at least 20,000 and a  $M_w$  of less than 125,000 is extruded through a high temperature spinneret (220°-335° C.) to form yarns which are hot-drawn at a temperature between about 115° and 132° C. The yarns produced by this process are particularly useful as industrial cordage.

6 Claims, No Drawings

## HIGH TENACITY POLYETHYLENE FIBERS AND PROCESS FOR PRODUCING SAME

This is a division, of application Ser. No. 848,168 filed Nov. 3, 1977, now U.S. Pat. No. 4,228,118.

### BACKGROUND OF THE INVENTION

#### A. Field of the Invention

This invention relates to high density polyethylene yarns having a tenacity of at least 12 grams per denier (gpd) and to a process for producing the same at commercially attractive spinning speeds. The term "spinning speed" as used herein means the velocity in meters per minute (m/min.) of freshly extruded fibers, that is, the velocity of the solidified molten polymer in fiber form before it is drawn. The polyethylenes from which the fibers are extruded are high density polyethylenes having a number average molecular weight ( $\bar{M}_n$ ) of at least 20,000 and a weight average molecular weight ( $\bar{M}_w$ ) less than 125,000. The term "high density polyethylene" is used herein in accordance with conventional terminology and means substantially linear polyethylene having a density of from 0.92 to 1.0 g/cm<sup>3</sup>. The term "fiber" as used herein means a single filament or a 25 yarn, that is, a bundle of filaments.

#### B. Description of the Prior Art

Polypropylene, nylon 6 and nylon 66 fibers are widely used in industry as cordage, for example, rope. Industrial cordage fibers normally have a tenacity ranging from about 6 to about 10 gpd and are commonly referred to as high tenacity fibers. There has been a continuing demand in the cordage industry to provide a lower cost high tenacity fiber suitable for cordage end uses. It is envisioned that such a fiber must meet three criteria in order to be competitive with the fibers presently used as cordage. First, the fiber must be produced from a fiber-forming material which is less expensive than polypropylene, nylon 6 or nylon 66. Secondly, the fiber must have a tenacity at least as high as the fibers presently used as industrial cordage and, preferably, a tenacity of at least 12 gpd. Lastly, the fiber must be capable of being produced at reasonably attractive spinning speeds. While it is generally recognized that polyethylene meets the first criterion, heretofore, it has not been possible to produce polyethylene fibers having a tenacity of at least 12 gpd at reasonable spinning speeds.

Most of the work that has been done to date and reported in the literature on polyethylene fibers is directed to processes for producing high modulus polyethylene fibers as a low cost substitute for glass and graphite fibers, which fibers have been traditionally used as the reinforcing material in composites. Such a process is described in U.S. Pat. No. 3,962,205 and West German Patent 2,650,747. The process involves extruding a high density polyethylene of a specified weight average molecular weight (i.e.  $\bar{M}_w$ ) and number average molecular weight (i.e.  $\bar{M}_n$ ) to form fibers which are cooled to a temperature of from 100° to 120° C. at the rate of from 1° to 15° C. per minute and then rapidly cooled. The fiber is then drawn at a temperature at least 40° C. below its melting point at a draw ratio of at least 18. This process however apparently must be operated at very slow spinning speeds due in part at least to the slow cooling step, for example, in the patents a 65 spinning speed of only about 4-5 meters per minute (m/min.) is illustrated. Moreover, applicants have been unable to produce high tenacity fibers (i.e. yarns having

a tenacity of 12 gpd or higher) from the particular polyethylenes specified in the U.S. patent even under conditions which would normally maximize tenacity. The German patent differs from the U.S. patent in that it 5 extends the useful polyethylenes to include those having a  $\bar{M}_w$  greater than 200,000 (e.g. 310,000 to 1,000,000), whereas the U.S. patent specified only those polyethylenes having a  $\bar{M}_w$  less than 200,000 and a  $\bar{M}_n$  less than 20,000. However, since the melt viscosity of a 10 polyethylene is directly proportional to its  $\bar{M}_w$ , fibers of the high  $\bar{M}_w$  polyethylenes disclosed in the German patent cannot be produced at commercially feasible spinning speeds by presently known means.

Therefore, it is an object of the present invention to 15 provide polyethylene yarns having a tenacity of at least 12 gpd and a process for producing the same at commercially feasible spinning speeds.

Other objects and advantages of the invention will 20 become apparent from the following detailed description thereof.

### SUMMARY OF THE INVENTION

In accordance with the foregoing objects, the present invention provides polyethylene yarns having a tenacity of at least 12 gpd. The invention also provides a process for producing such yarns or a single filament at commercially feasible spinning speeds, that is, at spinning speeds of at least 30 m/min. and, preferably, at least 50 m/min. The process comprises:

(1) extruding a high density polyethylene having a  $\bar{M}_n$  of at least 20,000 and a  $\bar{M}_w$  of less than 125,000 through a heated spinneret having at least one orifice to provide at least one molten stream, wherein said heated spinneret is maintained at a temperature between about 220° and 335° C.;

(2) solidifying each said molten stream in a quenching zone to form a fiber;

(3) withdrawing said fiber from said quenching zone at a velocity (i.e. spinning speed) of at least 30 m/min., and then

(4) hot-drawing said fiber at a given draw ratio while said fiber is in contact with a heated environment, wherein said heated environment is maintained at a temperature between 115° and 132° C., said temperatures, said velocity, and said draw ratio being correlated to provide a fiber having a tenacity of at least 12 gpd. The hot-drawing step may be accomplished inline (i.e. without take-up of the spun fiber) or the spun fiber may be taken-up and subsequently hot-drawn in a separate operation. The process may be employed to provide a monofilament or a yarn (bundle of filaments).

The process of the present invention is carried out under conditions which have been found by applicants to maximize the tenacities of polyethylene fibers. First, it is essential that the polyethylenes from which the fibers are produced have a  $\bar{M}_n$  of at least 20,000 and a density of at least 0.92 g/cm<sup>3</sup> and preferably at least 0.96 g/cm<sup>3</sup>. Secondly, it is also essential that the spinneret used in producing the fibers be maintained at a temperature between about 220° and about 335° C. Thirdly, the fibers must be hot-drawn at a temperature between 115° and 132° C. and at an optimum draw ratio. Lastly, the spinning speed and each of the foregoing conditions must be correlated to provide yarns having tenacities of at least 12 gpd. Under the foregoing conditions, the process can be carried out at commercially feasible spinning speed, for example, at spinning speeds of at

least 30 m/min. and as high as 700 m/min. by using polyethylenes which in addition to having the above properties also have a  $\bar{M}_w$  less than 125,000.

Heretofore, the  $\bar{M}_n$  property of polyethylenes has not been considered to be particularly significant in obtaining fibers of high tensile strength. In the past, the property thought to be the most important in obtaining polyethylene fibers of high tensile strength was the  $M_w$  property. Also, heretofore, high temperature spinnerets have not to applicants' knowledge been used in producing high tenacity polyethylene yarns. It is believed that the use of the right polyethylene and a high temperature spinneret in combination with optimum hot-drawing conditions are essential for producing polyethylene yarns having a tenacity of at least 12 gpd.

The fibers of the invention are particularly useful as cordage, for example, rope and the like where breaking strength is of primary importance.

#### DETAILED DESCRIPTION OF THE PREFERRED EMBODIMENTS

The yarns of the present invention have a tenacity of at least 12 gpd and are produced by the above-described process. The process comprises extruding a certain polyethylene through a high temperature spinneret having at least one orifice to provide one or more molten streams, each of which is solidified in a quenching zone. The number of molten streams corresponds to the number of orifices in the spinneret. The resulting yarn is withdrawn from the quenching zone at a given velocity and subsequently hot-drawn at a temperature between 115° and 132° C. and at an optimum draw ratio. The conditions under which the process is carried out are correlated to produce yarns having a tenacity of at least 12 gpd at a spinning speed of at least 30 m/min. It will be understood that more than one process variable has an effect on the tenacity of the drawn yarn. The following discussion will consider the effect of changing only one of these variables while holding the other variables constant.

High density polyethylenes useful in carrying out the process must have a  $\bar{M}_n$  of at least 20,000. When the  $\bar{M}_n$  is less than 20,000, yarns having a tenacity of at least 12 gpd are not obtainable at commercially feasible speeds. Preferably, the polyethylenes have a density of 0.96 g/cm<sup>3</sup> or higher and the  $\bar{M}_n$  is at least 22,000. In order to obtain high spinning speeds the polyethylenes must have a  $\bar{M}_w$  less than about 125,000. As with other polymers, the melt viscosity of polyethylenes increases with increasing  $\bar{M}_w$  values. Accordingly, the maximum possible spinning speed that may be used in carrying out the process is limited by the  $\bar{M}_w$  value of the particular polyethylene employed and is inversely proportional to the  $\bar{M}_w$  of the polyethylene. The spinning speed may be calculated by multiplying the velocity (V) of the molten polymer in the spinneret orifice and the jet stretch factor (JS), where JS is the amount of attenuation (or stretch) imparted to the molten streams between the spinneret and before their solidification in the quenching zone. The maximum spinning speed obtainable with a polyethylene of a given  $\bar{M}_w$ , where a yarn having a tenacity of at least 12 gpd is desired, is limited by both V and JS. V must not be so high as to cause melt fracture, a condition under which turbulence of the melt exists within the orifice and useful fibers can no longer be obtained. On the other hand, JS must not be so high that the tenacity of the drawn yarn is reduced to less than 12 gpd by reason thereof. Tenacity of the drawn

fiber increases with increasing JS to a maximum value and thereafter rapidly decreases with increase in JS. Accordingly, for a polymer of a given  $\bar{M}_w$  extruded at a given V, the tenacity of the drawn fiber can be maximized by selecting the appropriate spinning speed. While tenacity generally increases with increasing  $\bar{M}_w$  within the range of 60,000 to 125,000, the V<sub>max</sub> and JS<sub>max</sub> values decrease with increasing  $\bar{M}_w$  values. From experimental data in which conditions were selected to maximize tenacity the following formulas were derived to enable one to easily determine the maximum spinning speed (SS<sub>max</sub>) and jet stretch factor (JS<sub>max</sub>) that may be utilized in carrying out the process of this invention with a high density polyethylene of a given  $\bar{M}_w$  between 60,000 and 125,000:

$$(Formula 1) SS_{max} = 1858.4 - 2.7966 \times 10^{-2} \times \frac{1}{\bar{M}_w + 1.6703 \times 10^{-7} \times (\bar{M}_w)^2 - 3.8969 \times 10^{-13} \times (\bar{M}_w)^3}$$

$$(Formula 2) JS_{max} = 158.53 - 1.5387 \times 10^{-3} \times \frac{1}{\bar{M}_w} + 5.0393 \times 10^{-9} \times \frac{1}{(\bar{M}_w)^2} - 6.6848 \times 10^{-15} \times \frac{1}{(\bar{M}_w)^3}$$

In order to obtain yarns having a tenacity of 12 gpd, a high temperature spinneret must be used in carrying out the process. According to one embodiment of the invention, the molten polymer is extruded through a spinneret maintained at a temperature between about 220° and 335° C. into a quenching zone. At spinneret temperatures less than about 220° C., yarns having a tenacity of 12 gpd or higher are not obtainable and/or reasonable spinning speeds cannot be employed. On the other hand, the use of spinneret temperatures higher than about 335° C. causes degradation of the polymer and therefore are not desirable. According to another embodiment of the invention, a heated tube having an inside air temperature between 200° and 335° C. is positioned between the heated spinneret and the quenching zone. The tube is conveniently heated by electrical means and may be heated uniformly or different sections of the tube may be heated to different temperatures, for example, the upper half of the tube may be maintained at a higher or lower temperature than the lower half of the tube. Preferably, when a heated tube is employed, both the spinneret and heated tube are maintained at a temperature between 220° and 290° C. with a temperature between 260° and 280° C. being particularly preferred. While higher temperatures may be employed, such temperatures do not result in a significant increase in the tenacity of the drawn fiber. Although the use of a heated tube does not result in a significant increase in the tenacity of the drawn yarn, the use of such a tube facilitates spinning and packaging of the fibers. The heated tube normally may be positioned a short distance (e.g. 25 cm or less) from the spinneret and may be 50 cm. to 1 meter or more in length.

The molten streams upon moving away from the spinneret or, when used, from the heated tube are solidified in a quenching zone. Preferably, quenching of the molten streams is assisted by exposing the molten streams to transverse flowing air in a conventional manner. The air is conventionally at ambient temperature and at a velocity so as not to cause turbulence of the streams and/or solidified fibers. The molten streams attenuate as they move away from the spinneret in an amount corresponding to the jet stretch factor (JS).

According to one embodiment of the invention, the solidified fiber is taken-up on a bobbin without drawing at a take-up speed (spinning speed) of at least 30 m/min.

and preferably at least 50 m/min. This fiber is then used as the feed fiber in the hot-drawing step. Alternatively, the spinning and hot-drawing may be coupled, that is, carried out inline without intermediate take-up of the fiber.

In order to obtain yarns having a tenacity of at least 12 gpd, the process must be carried out under hot-drawing conditions which maximize the tenacity of the fiber. It has been found that the hot-drawing temperature (i.e. temperature of the heated environment) must be maintained at a temperature between about 115° and 132° C. if yarns having a tenacity of at least 12 gpd are to be obtained. Within this relatively narrow temperature range, the draw ratio is correlated with the particular temperature employed to obtain yarns having tenacities of at least 12 gpd. Normally, this draw ratio will be at least about 20:1. Fibers having the highest tenacity are produced when the hot-drawing temperature is between 124° and 132° C. and the draw ratio is at least 22:1. Normally, when the polyethylene fiber is hot-drawn at a given temperature between 115° and 132° C., the tenacity of the fiber increases with increasing draw ratio to a maximum value and thereafter remains substantially constant or decreases slightly with increasing draw ratio. It has been found that under most hot-drawing conditions this maximum tenacity value is obtained at a draw ratio ranging from about 20:1 to about 35:1 or higher. However, the modulus of the fiber continues to increase as the draw ratio increases beyond the draw ratio at which maximum tenacity is obtained. Accordingly, where the modulus of the fiber as well as the tenacity thereof is important, draw ratios higher than that required to obtain a fiber of maximum tenacity may beneficially be employed. The hot-drawing of the fiber may be accomplished in a conventional manner, such as, by passing the fibers into contact with a heated environment maintained at a temperature between 115° and 132° C. while drawing the fiber at an optimum draw ratio. The heated environment may consist of a heated inert gas such as air or nitrogen or a heated metal surface (e.g. hot shoe) over which the yarn passes or a heated fluid such as hot ethylene glycol. Also, a heated metal block, rectangular in shape, having a slot running along a surface thereof through which the fiber passes without contacting to the extent possible any surfaces of the block may be suitably used. The hot-drawing of the fiber may be accomplished in a conventional manner such as by passing the fiber with several wraps around a first and then a second pair of driven rolls, where the first pair of rolls is positioned before the fiber contacts the heated environment and the second pair of rolls afterwards and where the peripheral speed of the first pair of rolls ( $S_1$ ) and the peripheral speed ( $S_2$ ) of the second pair of rolls are correlated to give a desired draw ratio ( $S_2/S_1$  = draw ratio). The fiber is then taken-up in a conventional manner such as on to a bobbin under slight tension to facilitate packaging.

The foregoing discussion has been given from the standpoint of maximizing tenacity and spinning speeds. It will be apparent to those skilled in the art that certain processing conditions may be varied over a wide range without departing from the scope of this invention, such as, the manner in which the molten streams are quenched or the fiber is taken-up or the particular heated environment employed.

The following examples are given to further illustrate the invention but are not intended to in any way limit the scope thereof.

In the examples, the tenacity (gpd), elongation (%) and modulus (gpd) are measured on yarns composed of at least 8 filaments at 72% relative humidity and 25° C. on an Instron Tester (Instron Engineering Corporation, Canton, Mass.) providing a constant extension rate of 120% per minute with a gauge length of 25 cm being used. All values given in the examples are based on the average of four tests (breaks). The measured denier of the fiber, test conditions and sample identifications are fed to a computer before the start of the test. The computer records the load-elongation curve of the fiber sample until the sample is broken and the calculates and records tenacity, elongation and modulus.

#### EXAMPLE 1

This example illustrates the product of polyethylene fiber of the present invention.

Polyethylene having a density of 0.96 g/cm<sup>3</sup>, a  $\bar{M}_w$  of 84,000 and a  $\bar{M}_n$  of 25,200 was melted in a conventional melt extruder and extruded through an 8-hole spinneret at the rate of 2.4 g/min. to provide molten streams. Each hole (orifice) of the spinneret measured 9 mils (0.23 mm)  $\times$  12 mils (0.30 mm) (diameter/length). The spinneret was maintained at a temperature of 240° C. A heated tube having an inside air temperature of 260° C. and measuring 24 inches (61 cm) in length was positioned about 4 inches (10.2 cm) below the spinneret. The molten streams passed through the heated tube and then through a quenching zone measuring about 1 m in length where the molten streams solidified to provide fibers. In the quenching zone the molten streams were exposed to transverse flowing air (ambient temperature) for a distance of about 1 m. The velocity of the flowing air was adjusted so as not to cause turbulence of the molten streams. From the quenching zone the fiber was passed into contact with an air turbine guide (partial wrap), then passed with 4 wraps around a pair of rolls rotating at a peripheral speed of 44 m/min., and finally were wound up on a bobbin at constant tension by means of a tension guide at the same speed (i.e. 44 m/min.). The resulting bobbin of yarn was used as the feed yarn in the drawing operation. In the drawing operation, the yarn was unwound from the bobbin and passed with 10 wraps around a pair of rolls rotating at a peripheral speed of about 11 ft. (3.4 m)/min. The yarn was then passed over a 16 inch (40.6 cm) hot block maintained at a temperature of 126.7° C., then with 10 wraps around a pair of rolls rotating at a peripheral speed of 282 ft. (86 m)/min. to give a draw ratio of 25.7, and finally taken up at constant tension on a bobbin at the same speed (282 ft/min.). The tenacity, elongation-to-break and modulus of the yarn were determined and found to be 13.7 gpd/5.02%/428 gpd, respectively.

#### EXAMPLES 2-12

These examples are given to illustrate additional sets of conditions which may be used in carrying out the process of this invention. Certain of the conditions were varied from example to example to illustrate the effect thereof on tenacity. In each example the conditions were correlated to maximize tenacity.

Yarns were prepared using the apparatus, procedure and polyethylene described in Example 1. In each example air was used as the quench medium. In the hot-drawing step the draw ratio was varied from example to example by adjusting the peripheral speed of the pair of rotating rolls downstream from the hot block while maintaining the peripheral speed of the pair of rolls

upstream from the hot block at 3.4 m/min. The tenacity, elongation and modulus of each yarn were determined and are given in Table I along with the processing conditions employed for each example including Example 1.

neret) and procedure described in Example 1 was employed under the following set of conditions:

spinneret temperature—266° C.  
hot tube (length/temperature)—24 inches (61 cm)/125° C.

TABLE I

| EXAMPLE                 | 1     | 2     | 3     | 4     | 5     | 6     | 7     | 8     | 9     | 10    | 11    | 12    |
|-------------------------|-------|-------|-------|-------|-------|-------|-------|-------|-------|-------|-------|-------|
| Spinneret Temp. °C.     | 240   | 240   | 260   | 220   | 260   | 260   | 220   | 260   | 260   | 280   | 280   | 280   |
| Hot Tube, Temp. °C.     | 260   | 260   | 280   | 240   | 240   | 280   | 240   | 23    | 260   | 280   | 280   | 280   |
| Polym. Flow Rate g/min. | 2.4   | 2.4   | 2.4   | 2.4   | 2.4   | 2.4   | 2.4   | 2.4   | 2.4   | 5.0   | 5.0   | 7.8   |
| Spinning Speed m/min.   | 44    | 75    | 101   | 101   | 101   | 44    | 44    | 75    | 75    | 150   | 75    | 75    |
| Hot Block, Temp. °C.    | 126.7 | 128.9 | 127.8 | 127.3 | 127.8 | 127.8 | 127.8 | 127.6 | 127.7 | 127.7 | 128.7 | 128.2 |
| Draw Ratio              | 25.7  | 25.0  | 26.7  | 18.1  | 23.8  | 23.8  | 23.8  | 22.6  | 19.7  | 23.8  | 23.2  | 23.5  |
| Tenacity (gpd)          | 13.7  | 15.17 | 15.57 | 5.43  | 13.1  | 13.5  | 12.3  | 12.95 | 12.67 | 16.70 | 13.10 | 13.6  |
| Elong. %                | 5.02  | 5.23  | 5.10  | 7.35  | 5.64  | 5.20  | 3.91  | 6.24  | 7.10  | 4.60  | 5.94  | 5.08  |
| Modulus (gpd)           | 428   | 513   | 590   | 86    | 303   | 316   | 337   | 399   | 272   | 581   | 300   | 546   |

The results shown in Table I illustrate the effect of various sets of correlated processing conditions on the tenacities of the drawn yarns. For instance, Examples 1 and 2; 3 and 6; and 4 and 7 illustrate the effect of spinning speed on tenacity. In Example 4 a draw ratio of greater than about 11.3 could not be used without breaking the yarn. The resulting yarn in this example had a tenacity of only 5.43 gpd. In example 7 the spinning speed was reduced from 101 to 44 m/min. which permitted the use of a higher draw ratio (i.e. 23.8:1) whereby a yarn having a tenacity of 12.3 gpd was obtained. As shown by Examples 3 and 10, yarns of the highest tenacity were obtained when the spinneret was maintained at 260° or 280° C.

## EXAMPLE 13

This example illustrates the production of a monofila-

20 quench medium—air  
polymer flow rate—1.58 g/min.  
spinning speed—342 m/min.  
hot-draw (temperature/draw ratio)—126.8° C./23.18

## EXAMPLES 14-32

In these examples yarns were produced using the apparatus and procedure described in Examples 1-12 with the exception that in this instance the polyethylene had a  $M_n$  of 28,000, a  $M_w$  of 115,000 and a density of 0.96. The processing conditions were varied from example to example to demonstrate the effect thereof on the tenacity of the drawn yarns. The set of conditions used in each example is given in Table II. As in Examples 1-12, an 8-hole spinneret, each hole measuring 0.23 mm  $\times$  0.30 mm (diameter/length), was employed in each example.

TABLE II

| EXAMPLE                 | 14    | 15    | 16    | 17    | 18    | 19    | 20    | 21    | 22    | 23    | 24    |
|-------------------------|-------|-------|-------|-------|-------|-------|-------|-------|-------|-------|-------|
| Spinneret Temp. °C.     | 300   | 280   | 299   | 275   | 275   | 325   | 300   | 300   | 300   | 325   | 275   |
| Hot Tube, Temp. °C.     | 270   | 280   | 23    | 220   | 220   | 220   | 245   | 245   | 245   | 270   | 270   |
| Polym. Flow Rate g/min. | 2.4   | 2.4   | 2.35  | 2.35  | 2.35  | 2.35  | 2.35  | 2.35  | 2.35  | 2.35  | 2.35  |
| Spinning Speed m/min.   | 200   | 50    | 60    | 45    | 75    | 45    | 30    | 90    | 60    | 45    | 45    |
| Hot Block, Temp. °C.    | 125.6 | 128.8 | 127.7 | 127.5 | 127.1 | 127.7 | 127.8 | 127.8 | 127.9 | 127.6 | 127.4 |
| Draw Ratio              | 26.0  | 26.4  | 27.20 | 22.9  | 26.6  | 22.9  | 22.6  | 22.6  | 26.1  | 21.3  | 20.6  |
| Tenacity (gpd)          | 14.30 | 14.97 | 15.16 | 14.0  | 15.92 | 13.16 | 13.4  | 14.16 | 14.27 | 12.48 | 13.25 |
| Elong. %                | 5.07  | 4.76  | 4.69  | 5.77  | 4.69  | 5.93  | 5.98  | 5.19  | 4.55  | 6.39  | 6.21  |
| Modulus (gpd)           | 902   | 1043  | 831   | 759   | 1145  | 660   | 691   | 790   | 894   | 623   | 619   |
| EXAMPLE                 | 25    | 26    | 27    | 28    | 29    | 30    | 31    | 32    |       |       |       |
| Spinneret Temp. °C.     | 325   | 300   | 300   | 300   | 300   | 300   | 300   | 300   |       |       |       |
| Hot Tube, Temp. °C.     | 270   | 23    | 270   | 270   | 270   | 270   | 270   | 270   |       |       |       |
| Polym. Flow Rate g/min. | 2.35  | 4.8   | 4.8   | 4.8   | 4.8   | 4.8   | 4.8   | 4.8   |       |       |       |
| Spinning Speed m/min.   | 75    | 45    | 60    | 90    | 90    | 105   | 120   | 158   |       |       |       |
| Hot Block, Temp. °C.    | 127.9 | 127.0 | 127.8 | 128.5 | 128.5 | 127.8 | 127.0 | 127.0 |       |       |       |
| Draw Ratio              | 20.6  | 23.5  | 22.1  | 31.8  | 31.7  | 19.2  | 22.6  | 16.7  |       |       |       |
| Tenacity (gpd)          | 12.33 | 13.59 | 13.11 | 17.24 | 19.38 | 12.72 | 13.85 | 13.71 |       |       |       |
| Elong. %                | 5.25  | 5.79  | 5.75  | 3.70  | 3.86  | 6.83  | 5.65  | 6.93  |       |       |       |
| Modulus (gpd)           | 626   | 754.8 | 642   | 8.26  | 854   | 564   | 747   | 554   |       |       |       |

ment polyethylene fiber having a yarn tenacity of 13.99 gpd, an elongation-to-break of 5.49% and a modulus of 499 gpd (8 of the monofilaments were combined in the testing thereof).

In this instance, the polyethylene described in Example 1 was extruded through a spinneret having a single orifice measuring 25 mils (0.6 mm)  $\times$  50 mils (1.2 mm) (diameter/length). The apparatus (except from the spin-

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 65

## EXAMPLES 33-55

These examples illustrate the importance of utilizing a polyethylene having a  $\bar{M}_n$  of at least 20,000. In these examples a polyethylene having a  $M_n$  of 13,100, a  $\bar{M}_w$  of 86,700 and a density of 0.964 was melt spun into fiber using the apparatus and procedure described in Example 1. The processing conditions were varied from example to example in an effort to produce a yarn having a tenacity of 12 gpd or higher. In no instance could such a yarn be produced. The conditions used in each of the examples are given in Table III. In each instance a spinneret having six orifices each measuring 9 mils (0.23 mm)  $\times$  12 mils (0.30 mm) (diameter/length) was employed.

15

TABLE III

| EXAMPLE                 | 33    | 34    | 35    | 36    | 37    | 38    | 39    | 40    | 41    | 42    | 43    | 44    |
|-------------------------|-------|-------|-------|-------|-------|-------|-------|-------|-------|-------|-------|-------|
| Spinneret Temp. °C.     | 294   | 294   | 275   | 275   | 325   | 325   | 251   | 300   | 298   | 298   | 325   | 275   |
| Hot Tube, Temp. °C.     | 23    | 23    | 220   | 220   | 220   | 220   | 245   | 245   | 245   | 245   | 270   | 270   |
| Polym. Flow Rate g/min. | 2.6   | 2.6   | 2.6   | 2.6   | 2.6   | 2.6   | 2.6   | 2.6   | 2.6   | 2.6   | 2.6   | 2.6   |
| Spinning Speed m/min.   | 60    | 80    | 60    | 100   | 60    | 100   | 80    | 40    | 120   | 80    | 60    | 60    |
| Hot Block, Temp. °C.    | 124.1 | 124.0 | 125.0 | 125.0 | 125.0 | 125.0 | 125.0 | 125.0 | 125.0 | 123   | 123.4 | 123.4 |
| Draw Ratio              | 20.86 | 20.86 | 20.86 | 17.62 | 22.25 | 21.33 | 12.98 | 22.56 | 14.68 | 19.78 | 22.87 | 22.41 |
| Tenacity (gpd)          | 8.99  | 10.43 | 10.12 | 8.82  | 10.0  | 9.58  | 7.62  | 9.74  | 7.77  | 9.51  | 9.15  | 10.32 |
| Elong. %                | 5.45  | 5.78  | 6.03  | 6.40  | 5.69  | 5.35  | 9.14  | 5.43  | 7.79  | 6.16  | 5.15  | 5.80  |
| Modulus (gpd)           | 289   | 301   | 293   | 232   | 299   | 307   | 149   | 301   | 162   | 264   | 294   | 319   |
| EXAMPLE                 | 45    | 46    | 47    | 48    | 49    | 50    | 51    | 52    | 53    | 54    | 55    |       |
| Spinneret Temp. °C.     | 275   | 325   | 300   | 300   | 298   | 300   | 300   | 300   | 300   | 300   | 300   |       |
| Hot Tube, Temp. °C.     | 270   | 270   | 23    | 270   | 270   | 270   | 270   | 270   | 270   | 270   | 270   | 23    |
| Polym. Flow Rate g/min. | 2.6   | 2.6   | 4.7   | 4.7   | 4.7   | 4.7   | 4.7   | 4.7   | 4.7   | 4.7   | 4.7   | 4.7   |
| Spinning Speed m/min.   | 100   | 100   | 60    | 60    | 80    | 100   | 120   | 140   | 160   | 207   | 120   |       |
| Hot Block, Temp. °C.    | 124.7 | 124.6 | 126.2 | 125.7 | 124.1 | 125.8 | 125.6 | 125.6 | 125.8 | 124.7 | 124.9 |       |
| Draw Ratio              | 20.1  | 16.7  | 21.8  | 23.2  | 24.1  | 21.5  | 20.0  | 16.5  | 19.5  | 12.7  | 18.2  |       |
| Tenacity (gpd)          | 9.17  | 8.05  | 9.14  | 10.95 | 10.68 | 10.54 | 10.33 | 9.36  | 10.13 | 7.40  | 9.55  |       |
| Elong. %                | 5.37  | 6.88  | 5.82  | 5.65  | 5.19  | 6.13  | 5.83  | 8.10  | 6.22  | 9.78  | 6.57  |       |
| Modulus (gpd)           | 283   | 220   |       |       |       |       |       |       |       |       |       |       |

The results in Table III show that it is essential to 40 obtaining yarn having a tenacity of at least 12 gpd that the process be carried out using a high density polyethylene having a  $\bar{M}_n$  of at least 20,000. It will be appreciated that the polyethylene used in the instant examples had an  $\bar{M}_w$  of 86,700 which is higher than the  $\bar{M}_w$  of the 45 polyethylene used in Examples 1-13 ( $\bar{M}_w$  of 84,000), wherein yarns having a tenacity of 12 or more gpd were obtained.

## EXAMPLE 56

Based on the results obtained in Examples 33-55 a further experiment was carried out to determine, if under optimum conditions, a yarn having a tenacity of 12 or more gpd could be obtained at some draw ratio between 20:1 and 30:1.

In this experiment two as-spun yarns were prepared from the polyethylene described in Examples 33-55 under optimum spinning conditions. Samples of each of the as-spun yarns were then hot-drawn at different draw ratios increasing from about 20:1 until a draw 60 ratio of about 30:1 was obtained at an optimum hot-drawing temperature (124°-125° C.) in an effort to provide a yarn having a tenacity of 12 gpd or higher.

The as-spun yarns were prepared using the apparatus and procedure described in Examples 33-55 under the 65 following conditions:

spinneret temperature—299°  $\pm$  1° C.

hot tube (length/temperature)—24 inches/270° C.

quenching medium—air  
polymer flow rate—4.7 g/min.

The as-spun yarns were then hot-drawn using the apparatus and procedure described in Examples 33-55. In the hot-drawing operation each yarn sample was withdrawn from the feed bobbin at 11 ft. (3.4 m)/min., passed over the 16 inch-hot block and collected at a speed so as to give the draw ratios shown in the following table. The hot block was maintained at a temperature of 124°-125° C. This temperature was selected as being the optimum hot-drawing temperature under the conditions of this experiment. The tenacity, elongation and modulus of each yarn sample were determined and are also given in the table.

TABLE IV

| Fiber | Draw Ratio | Tenacity (gpd) | Elong. % | Modulus (gpd) |
|-------|------------|----------------|----------|---------------|
| 1     | 23.18      | 10.95          | 5.65     | 344           |
|       | 23.71      | 10.09          | 5.22     | 341           |
|       | 25.5       | 10.23          | 5.11     | 353           |
|       | 25.5       | 9.47           | 4.55     | 348           |
|       | 26.1       | 9.26           | 4.44     | 350           |
|       | 26.27      | 8.17           | 3.60     | 419           |
|       | 27.19      | 10.52          | 4.29     | 409           |
| 2     | 19.94      | 9.76           | 6.76     | 259           |
|       | 22.1       | 10.12          | 5.80     | 303           |
|       | 23.18      | 10.38          | 5.70     | 320           |
|       | 24.11      | 10.68          | 5.19     | 357           |
|       | 26.12      | 10.96          | 4.92     | 389           |
|       | 28.68      | 10.34          | 3.78     | 452           |
|       | 30.6       | 10.59          | 3.79     | 483           |

55

The results of this example further demonstrates the necessity of using a polyethylene having a  $\bar{M}_n$  of at least 20,000 if yarns having a tenacity of at least 12 gpd are to be obtained. While  $\bar{M}_w$  is important with regard to spinning speeds and has some effect on tenacity, the results of this example and the previous examples clearly demonstrate that employing polyethylenes having a  $\bar{M}_n$  of at least 20,000 is essential in obtaining fibers at 12 or more gpd regardless of the  $\bar{M}_w$  value of the polyethylene.

## EXAMPLE 57

This example illustrates carrying out the process of this invention at relatively high drawing speeds.

In the example as as-spun yarn was prepared under the same spinning conditions described in Example 16 using an eight-hole spinneret, each hole measuring 9 mils (3.4 mm)  $\times$  10 mils (2.54 mm). Samples of the as-spun yarn were hot-drawn using the apparatus and procedure described in Example 1 under the following conditions given in Table V, wherein  $S_1$  represents the speed of the pair of rolls upstream from the hot block and  $S_2$  represents the speed of the pair of rolls downstream from the hot block (drawing speed):

TABLE V

| Yarn Sample # | $S_1$<br>m/min. | $S_2$<br>m/min. | Draw Ratio<br>to 1 | Hot Block<br>Temp. °C. | Tenacity<br>gpd | Elong.<br>% | Modulus<br>gpd |
|---------------|-----------------|-----------------|--------------------|------------------------|-----------------|-------------|----------------|
| 1             | 6.7             | 191.7           | 28.6               | 127.1                  | 14.5            | 3.77        | 663            |
| 2             | 9.1             | 228.9           | 25.0               | 127.1                  | 14.4            | 4.38        | 578            |
| 3             | 10.8            | 274.0           | 25.3               | 127.1                  | 15.7            | 3.77        | 691            |

The results in Table V show that the hot-drawing step may be carried out at a relatively high drawing speed. The drawing speed was limited in this example only by virtue that the winder was not capable of running at take-up speeds higher than 274 m/min. Based on the experiment of this example, it is believed that drawing speeds considerably higher than 500 m/min. could be successfully utilized. Thus, the process can be carried out using commercially feasible spinning and drawing speeds whereby the spinning and drawing could be

accomplished in line without intermediate take-up of the yarn.

We claim:

1. Fibers consisting of a polyethylene having a  $M_n$  of at least 20,000, a  $M_w$  of less than 125,000, a density of between 0.92 and 1.00 grams per cubic centimeter, said fibers having a tenacity of at least 12 grams per denier and a modulus of at least 272 grams per denier when measured at 72% relative humidity and 25° C. on a 10 bundle of at least 8 filaments using a gauge length of at

least 25 centimeters.

2. The fibers of claim 1 wherein said  $M_n$  is at least 22,000.
3. The fibers of claim 1 wherein said density is at least 0.96 grams per cubic centimeter.
4. The fibers of claim 1 wherein said tenacity is at least 15 grams per denier.
5. The fibers of claim 1 in the form of a monofilament.
6. The fibers of claim 1 in the form of a yarn consisting of a bundle of filaments.

\* \* \* \* \*

30

35

40

45

50

55

60

65